

## UNITED STATES PATENT OFFICE.

ALBERT BEIL, OF HOCHST-ON-THE-MAIN, AND WILHELM ADOLF MEYER, OF HERSFELD, GERMANY, ASSIGNEES TO A. RECHBERG GESELLSCHAFT MIT BESCHRANKTER HAFTUNG AND GEORG BRAUN GESELLSCHAFT MIT BESCHRANKTER HAFTUNG, BOTH OF HERSFELD, GERMANY.

## PROCESS FOR EXTRACTING FATS FROM TEXTILES.

No Drawing. Application filed March 11, 1926, Serial No. 94,095, and in Germany March 18, 1925.

The removal of fats from textiles by means of organic extraction agents is a problem which has often been discussed without, hitherto, a generally utilizable solution being found. Consequently it continued to be effected, almost without exception, by means of aqueous alkaline treatment. It is quite obvious that the removal of fat by organic solvents would be given the preference, if it were possible to carry out the de-fatting without danger of fire or explosion; under the utmost possible care to prevent deterioration of the fibres; without danger to the necessary apparatus and, above all, economically.

Methylenechloride has been shown to satisfy these requirements in a surprisingly perfect manner. Its employment as solvent forms therefore the subject of the present invention.

Chlorinated hydrocarbons have been repeatedly suggested for the de-fatting of textiles, firstly on account of their safeness in respect of fire, but also because the de-fatting is accompanied by very considerable improvement of the fibres. For example in the de-fatting of raw wool the fat of the surface only is dissolved out while the interior of the fibres remains undisturbed and the fibres retain, therefore, their resiliency and pliability.

The hydrocarbons employed hitherto all exhibit the disadvantage that in consequence of the catalytic formation of hydrochloric acid gas they damage the apparatus, a disadvantage which has hitherto not been successfully obviated. In contradistinction thereto methylenechloride is distinguished by an extraordinary resistance in respect of action thereon by heated contact substances, a circumstance which qualifies methylenechloride to serve excellently as a de-fatting agent. In addition the low boiling point of methylenechloride is also favorable since the heating of the apparatus does not need to be too intense.

The low boiling point of methylenechloride is also of advantage, in another direction, for the de-fatting of textiles. With many textiles, such as for example wool and silk, the heating for the driving off of the solvent must, as far as possible, not exceed 50° C. which is not feasible with the solvents of higher boiling point. Even if a vacuum is employed it is not possible, in the case of the solvents of higher boiling point to prevent, if the said solvents are to be removed completely, a portion of the material treated from being too strongly heated, and, in this manner, becoming brittle and weak. Insufficient heating, however, results, with the very voluminous textiles, in considerable quantities of solvent remaining in the material and being lost.

On account of its stability towards decomposing influences and because it can easily be removed without residue from the material to be de-fatted the employment of methylene-chloride for the de-fatting of textiles is economically feasible in contradistinction to the chlorinated hydrocarbons recommended heretofore.

*Example.*—1000 kilograms of raw-wool is treated once or several times with say from 6000 to 8000 liters of liquid methylenechloride in a rotary extraction apparatus of 10 cubic meters capacity. After drawing off the major portion of the solvent and dissolved fats, hot water at 50° C. is caused to flow through the heating jacket of the extractor and the apparatus is rotated quite slowly. Such heating drives off a large portion of the solvent retained by the wool. The residue of the solvent is then removed with the assistance of a vacuum.

What we claim as new and desire to secure by Letters Patent is:

1. In a method of defatting textiles by means of volatile solvents, the step of treating such textiles with liquid methylenechloride.
2. A method of defatting textiles which

2  
consists in subjecting such textiles to the solvent action of liquid methylenechloride, drawing off the major portion of the solvent and dissolved fats, subsequently heating the textiles to temperatures not exceeding 50° C. to volatilize and remove therefrom the major portion of the solvent retained by the textiles, and finally applying a vacuum to re-

move the residual solvent from such textiles.

In testimony that we claim the foregoing as our invention, we have signed our names this 26th day of February, 1926.

ALBERT BEIL.  
WILHELM ADOLF MEYER.